

# UNITED STATES PATENT OFFICE.

HUBERT A. MYERS, OF TOLEDO, OHIO, ASSIGNEE TO THE HUBERT A. MYERS COMPANY, OF TOLEDO, OHIO, A CORPORATION OF OHIO.

## MOLD AND METHOD OF TREATING SAME.

1,427,926.

Specification of Letters Patent. Patented Aug. 29, 1922.

No Drawing.

Application filed August 26, 1920. Serial No. 408,969.

To all whom it may concern:

Be it known that I, Hubert A. Myers, a citizen of the United States, and a resident of Toledo, in the county of Lucas and State of Ohio, have invented a certain new and useful Mold and Method of Treating Same; and I do hereby declare the following to be a full, clear, and exact description of the invention, such as will enable others skilled in the art to which it appertains to make and use the same.

This invention relates to the casting of metals and it particularly has for its object to so treat or prepare metal molds that complete castings having smooth surfaces may be formed.

In casting certain metals, particularly ferrous metals, in metal molds, such as iron molds, the metal of the casting will sometimes adhere to and cause pitting of the mold and of the casting. To overcome this it has been customary to line or coat the molds with a composition of graphite, clay, silica or other similar material. By my invention adherence between the casting and the mold and pitting of the mold and the casting are prevented by surfacing the mold with a metal having a melting point below that of the metal of the mold. This may be accomplished by heating the mold or the metal above the melting point of the metal, or heating both the mold and the metal and bringing the two into contact with each other at the molding surfaces. Intimate contact between the two may be brought about by rubbing the metal while in a molten state into the molding surface while the mold is at a temperature above the melting point of the metal.

In casting ferrous metals I have found that zinc is particularly of value as a lining to the mold as it fills the pores of the iron mold and forms a somewhat permanent coating that will permit the formation of a number of castings without retreatment of the mold.

When the mold has been heated to the desired extent zinc, or other suitable metal having a fusion point lower than that of the metal of the mold, is melted by contact with the hot mold, or in some other manner, and deposited thereon. It is then rubbed thoroughly into the surface pores of the

mold, preferably by a brush having metallic bristles, so that the mold surface is thoroughly impregnated and surfaced with the metal.

It is found in practice that a mold, ladle, crucible, or other metallic article treated in this manner will effectually prevent the sticking of molten metal thereto and that having once been treated the article may be repeatedly filled with molten metal without resurfacing with the metal having a low fusion point.

While I have described a particular method of applying a metal having a low melting point to the molding surfaces of the mold, it will be understood that it may be applied in other ways without departing from the spirit of the claims.

I claim:

1. The method of treating the surface of a metal article to prevent adherence of molten metals thereto, which consists in rubbing into the surface molten metal having a melting point lower than that of the metal of the article.

2. The method of treating the surface of a metal article to prevent adherence of molten metals thereto, which consists in rubbing into the surface of the article by the use of a brush having metal bristles, a molten metal having a melting point less than that of the metal of the article.

3. The method of treating the surface of a metal article to prevent adherence of molten metals thereto, which consists in rubbing molten zinc into the surface of the article.

4. The method of treating molds to prevent pitting of the mold and the casting, which consists in heating the mold and while hot rubbing zinciferous material over the face and into the pores of the casting surface of the mold, the mold being heated.

5. The method of treating metal molds to prevent sticking of molten metal to be cast therein, which consists in applying a metal to the heated molding surface of a mold, the mold being heated to a temperature to melt the applied metal, and then thoroughly rubbing the applied metal into the mold surface.

6. The method of treating metal molds to prevent sticking of molten metal thereto, which consists in heating the mold and

while hot rubbing zinc over the face and into the pores of the casting surface of the mold, the mold being heated to a zinc melting temperature.

5 7. The method of preparing a ferrous mold for forming ferrous castings, which consists in rubbing zinciferous material into the surface of the mold.

10 8. The method of preparing a ferrous mold for forming ferrous castings, which

consists in rubbing zinc into the surface of the mold.

9. The method of preparing a ferrous mold for forming ferrous castings, which consists in rubbing molten zinc into the surface of the mold. 15

In testimony whereof, I have hereunto signed my name to this specification.

HUBERT A. MYERS.